

# United States Patent

[19]

Tada et al.

[11] 3,931,430

[45] Jan. 6, 1976

[54] **METHOD OF DESENSITIZING A PRESSURE  
SENSITIVE RECORDING SHEET AND THE  
PRODUCT THEREOF**

[75] Inventors: **Tomonori Tada; Akira Shiono**, both  
of Osaka, Japan

[73] Assignee: **Kanzaki Paper Mfg. Co. Ltd.**,  
Tokyo, Japan

[22] Filed: **Nov. 7, 1973**

[21] Appl. No.: **413,437**

[30] **Foreign Application Priority Data**

Nov. 11, 1972 Japan ..... 47-113377

[52] **U.S. Cl.** ..... **428/195; 427/146; 427/150;**  
427/151; 428/211

[51] **Int. Cl.<sup>2</sup>** ..... **B41M 5/02**

[58] **Field of Search** ..... 117/36.7, 36.8; 427/146,  
427/150, 151; 428/195, 199, 211

[56] **References Cited**

UNITED STATES PATENTS

2,654,673 10/1953 Steinhardt ..... 106/22

|           |        |              |            |
|-----------|--------|--------------|------------|
| 2,730,456 | 1/1956 | Green et al. | 117/36.1   |
| 2,730,457 | 1/1956 | Green et al. | 117/36.8   |
| 3,809,668 | 5/1974 | Yarian       | 260/33.4 U |

*Primary Examiner*—Thomas J. Herbert, Jr.

*Assistant Examiner*—Bruce H. Hess

*Attorney, Agent, or Firm*—Cushman, Darby &  
Cushman

[57]

## ABSTRACT

The pressure sensitive recording sheet is partially de-sensitized by applying an improved desensitizer to a predetermined area thereof. The improved desensitizer comprises a reaction product produced by the reaction of ammonia, amines, diamines or polyamines with glycidyl esters or glycidyl ethers. The improved desensitizer is hydrophobic and soluble in an oil vehicle.

**9 Claims, No Drawings**

**METHOD OF DESENSITIZING A PRESSURE  
SENSITIVE RECORDING SHEET AND THE  
PRODUCT THEREOF**

**BACKGROUND OF THE INVENTION**

This invention relates to a method of desensitizing a pressure sensitive recording sheet and more particularly, to spot-desensitizing of a sheet sensitized with organic or inorganic color forming reactant acid materials which act as electron acceptor in an electron-donor-acceptor color-forming reaction. The invention also relates to desensitized sheets obtained by such desensitization.

There are known several types of pressure-sensitive recording system utilizing an electron donor-acceptor color-forming reaction between a colorless chromogenic material and a color forming reactant acid material. The colorless chromogenic material and the color forming reactant acid material are hereinafter referred to as "color former" and "color acceptor", respectively. Those pressure-sensitive recording systems comprise a support sheet having, disposed on at least one surface thereof, micro capsules containing oil droplets in which a color former is dissolved and/or a color acceptor capable of producing color when brought into reactive contact with the color former.

For example, U.S. Pat. No. 2,730,456 discloses a transfer-copy system wherein minute oil droplets in which a color former is dispersed or dissolved are encapsulated and coated onto a transfer sheet. The color former is thereafter transferred to a receiving sheet by rupturing said capsules. The underlying receiving sheet has a color reactant coating thereon containing a color acceptor which will react with the color former causing a visible colored mark at points where the microcapsules have been ruptured and the color former has been transferred. In case when multiple copies are needed at least one intermediate copy sheet having said micro-capsules and said color acceptor on the opposite surfaces thereof, respectively, is interposed between the upper copy sheet and the underlying copy sheet.

U.S. Pat. No. 2,730,457 discloses another type of a pressure-sensitive record sheet. In this pressure-sensitive record sheet, there are disposed on one surface of the same sheet both the color acceptor and the capsules containing oil droplets in which the color former is dissolved. This record material is known as a "self contained" system.

It is known to locally apply a desensitizer in advance onto the color-acceptor-coated surface in order to inactivate color-forming reactivity of the color former on the area where color-forming reaction is not required. The desensitizer may also be applied locally onto the color-acceptor-coated surface where a color image has been produced in order to erase the image.

Desensitizers which have been conventionally used are polyethylene glycol, glycerol, dodecyl trimethylammonium chloride, dodecyl amine, dodecyl dimethylamine, N,N-bispolyoxyethylene alkylamine, N,N,N-trispolyoxyethyleneamine, N,N,N'-trispolyoxyethylene N-alkylenediamine, N,N,N',N'-tetrakispolyoxyethylene alkylenediamine, N-alkyl-N,N',N',N'-trimethylalkylenediamine, etc. Among those desensitizers, ethylene oxide adducts of amine, diamine and polyamine are particularly superior in the desensitizing effect, but those adducts are not suitable for offset printing because hydrophobic vehicle can not be used in making

ink due to many hydrophilic groups of those adducts. In case that the pressure-sensitive recording sheet which is desensitized with the above mentioned adducts is placed in the condition of a high temperature and a high humidity, hygroscopic phenomenn by hydrophilic desensitizer becomes more remarkable and therefore the desensitizer applied onto the area where color-forming reaction is required migrates so far to the adjacent areas where color-forming reaction is not required, with the result that the ability of color-forming reaction at such the adjacent areas is lowered. In addition, as capsules on the back surface or the adjacent sheet are left in the extrodinary high humidity because of the hygroscopic property thereof, the spontaneous rupture of capsules will occur easily.

Recently, organic compounds such as aromatic carboxylic acids or polymers of organic acids such as phenol-formaldehyde resin which are more hydrophobic than inorganic solid acids have been used as color acceptor. For example, DT-OS 2147585, 2152765 and 2242250 disclose that the mixture of aromatic carboxylic acid derivatives such as benzoic acid, salicylic acid or derivatives of which with metal compounds such as metal oxide, metal hydroxide and metal carbonate; or metallic salts of above aromatic carboxylic acid derivatives can be used as color acceptor. It is also suggested in DT-OS 2148427 to use the mixture or copolymer of aromatic carboxylic acid, and aldehyde or acetylene with metallic compounds, and in DT-PS 2152763 to use metallic salts of the said polymer.

The above-mentioned conventional desensitizers are disadvantageous in that they remain sticky for a long time because of the poor affinity for the said organic acids and polymers thereof. Long chain alkyl-dimethyl amine and N-long chain alkyl-N,N',N'-trimethylalkylenediamine are rather hydrophobic but they have an undesirable smell inherent to amines. Especially, long chain alkyl dimethylamine does not show a satisfactory desensitizing effect.

The primary object of the invention is to provide a new and improved method for desensitizing a pressure sensitive recording sheet in which the above mentioned disadvantages with conventional desensitizers can be avoided and an excellent desensitizing effect is obtained.

Another object of the invention is to provide a new desensitizer which is hydrophobic and well soluble in oil vehicle to make an ink for offset printing use.

A further object of the invention is to provide an improved desensitizer which has a good affinity to the color acceptor coating layer which is made of an organic acid or polymer thereof.

A still further object of the invention is to provide an improved desensitizer ink which is superior in both inksetting and migration-resistance.

One of other objects of invention is to provide an improved desensitizer for the pressure sensitive recording sheet which is odorless.

It is also one of the objects of the invention to provide a partly desensitized, pressure sensitive recording sheet in which migration of the desensitizer applied to the sheet hardly occurs even in condition of a high temperature and a high humidity so that capsules containing oil droplets may be prevented from spontaneous rupture at the area adjacent to the area to which the desensitizer is applied.

## SUMMARY OF THE INVENTION

According to the invention the pressure sensitive recording sheet is desensitized by applying an improved desensitizer to a predetermined area thereof. The improved desensitizer comprises a reaction product produced by the reaction of ammonia, primary or secondary monoamines, primary or secondary diamines, or, primary or secondary polyamines with glycidyl esters or glycidyl ethers. The desensitizer is preferably applied in the form of an ink with an oil vehicle to a predetermined area of the pressure sensitive recording sheet.

The area of a pressure sensitive recording sheet to which the desensitizer according to the invention is applied is completely desensitized so that no color image is produced at this area even if any pressure is applied thereto. The reaction products produced by adding glycidyl esters or glycidyl ethers to active hydrogen of ammonia, monoamines, diamines and polyamines have an unexpectedly excellent desensitizing function. The above mentioned reaction products becomes more hydrophobic and more soluble in oil vehicles according as the molecular weight increases. Accordingly it is possible to prepare an ink for offset printing use by dissolving any of those reaction products in an oil vehicle. The reaction products according to the invention have a good affinity to the color acceptor coating layer which is made of an organic acid or polymer thereof and are superior in both ink-setting and migration-resistance. The reaction products described are odorless.

In the pressure sensitive recording sheet which is partly desensitized according to the invention, migration of the desensitizer applied to the sheet hardly occurs even in condition of a high temperature and a high humidity so that capsules containing oil droplets may be prevented from spontaneous rupture at the area adjacent to the area to which the desensitizer is applied.

## DETAILED DESCRIPTION OF THE INVENTION

According to the invention a reaction product produced by adding glycidyl esters or glycidyl ethers to active hydrogen of ammonia, primary or secondary monoamines, primary or secondary diamines, and, primary or secondary polyamines. Among the reactant amines there may be primary or secondary alkylamine, primary or secondary alkenylamine, primary or secondary cyclicamine, primary or secondary arylamine, etc. Particularly and preferably they are exemplified by methylamine, dimethylamine, ethylamine, diethylamine, butylamine, dibutylamine, allylamine, diallylamine, cyclohexylamine, cyclopentylamine, benzylamine, ethylenediamine, propylenediamine, hexamethylenediamine, diethylenetriamine, triethylenetetramine, 1,4-diaminocyclohexane, xylylenediamine, bis(3-methyl-4-amino cyclohexyl)methane, N-amino-propylcyclohexylamine, N-dodecylethylene-diamine, N-hexadecylethylenediamine, N-Octylpropylenediamine.

mine, N-dodecylpropylene-diamine, N-tetradecylpropylenediamine, N-stearylpropylenediamine, N-decyldiethylenetriamine, N-hexadecyl diethylenetriamine, N-dodecyltriethylenetetramine, N-octyltripropylenetetramine, N-decyltripropylenetetramine, piperazine, N-aminoethylpiperazine, N-aminopropylpiperazine, N-aminopropylmorpholine, N,N'-diaminopropylpiperazine, tris(N-aminopropyl)isocyanurate, etc.

10 Among useful glycidyl ethers or glycidyl esters there are alkylglycidylethers such as n-butylglycidylether, iso-butylglycidylether, hexylglycidylether, hexadecylglycidylether, etc., cycloalkylglycidylether such as cyclohexylglycidylether, etc., arylglycidylether such as phenylglycidylether, benzylglycidylether, o-phenyl-phenol-glycidylether, cinnamylglycidylether, etc., alkenylglycidylether such as allylglycidylether, crotylglycidylether, etc., glycidylalkylate such as glycidylbutylate, glycidylcaproate, glycidylcaprylate, glycidyllaurate, etc., glycidylalkenate such as glycidylmethacrylate, glycidylacrylate, glycidyl-crotonate, etc., and glycidylarylate such as glycidylbenzoate, glycidyl- $\alpha$ -benzylacrylate, glycidylbenzylacetate, etc.

25 The reaction products described therein may be obtained by heating the reaction system of ammonia or amines with glycidylether or glycidylester. The reactants react almost quantitatively, easily and in a short time. The desensitizer containing the reaction products thus obtained can be used in the various forms of ink 30 for letterpress, gravure, offset and flexographic printing, of solution to be sprayed obtained by dissolving in a proper solvent, and of solid obtained by mixing and temper with paraffin, japan wax and white pigment.

As vehicles for preparation of a desensitizing ink,  
35 there may be included drying oils such as linseed oil  
and soybean oil; synthetic drying oils such as copoly-  
merization oil of drying oil and styrene, dehydrated  
castor oil and urethanated oil; synthetic resins such as  
alkyd resin, polyester resin, polyamide resin and maleic  
40 acid resin; and mixture thereof.

Without limiting this invention, the following examples are given to illustrate the model of operation.

### EXAMPLE 1

45 32.6g (0.1 mol.) of N-stearylpropylenediamine (MW=326) was heated to 80°C to melt in a four neck flask which had a reflux condenser, a thermometer and stirrer. To the above melt, 35g (0.307 mol.) of allyl-glycidylether (MW=114) was added drop by drop. As 50 the reaction was exothermic, heating was stopped and allylglycidylether was added drop by drop at such speed that the system was kept in the temperature range of 80°–110°C. Then the system was heated at 110°C for 30 minutes and then excess allylglycidylether was removed by distillation. Finally, pale yellow 55 and viscous N-stearyl-N,N',N'-tris(2-hydroxy-3-allyloxypropyl)propylenediamine having the following formula was obtained.



## EXAMPLE 2

24.1g (0.1 mol.) of hexadecylamine (NW=241) and 23.5g (0.206 mol.) of allylglycidylether (MW = 114)

were allowed to react with each other in the same manner as in Example 1 and thereby N,N-bis(2-hydroxy-3-allyloxypropyl)N-hexadecylamine having the following formula was obtained.



## EXAMPLE 3

32.6g (0.1 mol.) of N-stearylpropylenediamine (NW=326) and 46g (0.307 mol.) of phenylglycidylether (MW=150) were allowed to react with each other in the same manner as in Example 1 and thereby N-stearyl-N,N',N'-tris(2-hydroxy-3-phenoxy-

propyl)propylenediamine having the following formula was obtained.



## EXAMPLE 4

32.6g (0.1 mol.) of N-stearylpropylenediamine (MW=326) and 43.5g (0.306 mol.) of glycidylmethacrylate (MW=142) were allowed to react with each

65

other in the same manner as in Example 1 and thereby N-stearyl-N,N',N'-tris(2-hydroxy-3-methacryloyloxypropyl) propylenediamine having the following formula was obtained.



## EXAMPLE 5

32.7g (0.1 mol.) of N-hexadecyltriethylene triamine (MW=327) and 53g (0.408 mol.) of butylglycidylether (MW=130) were allowed to react with each other in the same manner as in Example 1 and thereby N-hexadecyl-N,N',N',N'-tetrakis(2-hydroxy-3-butyoxypropyl)diethylenetriamine having the following formula was obtained.



## EXAMPLE 6

1 mol. of N-decyltripropylene tetramine and 5 mol. of benzyl-glycidylether were allowed to react with each other in the same manner as in Example 1 and thereby the compound having the following formula was obtained.



propyl)propylenediamine having the following formula was obtained.

45

## EXAMPLE 7

1 mol. of N-aminoethylpiperazine and 3 mol. of glycidylcaprylate were allowed to react with each other in the same manner as in Example 1 and thereby the compound having the following formula was obtained.



60

## EXAMPLE 8

1 mol. of triethylenetetramine and 6 mol. of cyclohexylglycidylether were allowed to react with each other in the same manner as Example 1 and thereby the compound having the following formula was obtained.





6. The method of claim 1, wherein said step of applying comprises dissolving said reaction product in a solvent to form a solution and spraying said solution.

7. The method of claim 1, wherein said step of applying comprises using said reaction product as a solid form wherein the densitizer is mixed and tempered with paraffin, japan wax and white pigment.

8. A partly desensitized, pressure sensitive recording sheet which is obtained according to the method defined in claim 1.

9. A method of desensitizing a pressure sensitive recording sheet comprising applying to a predetermined area of the pressure sensitive recording sheet a desensitizer which comprises a reaction product produced by the reaction of (1) ammonia, alkylamines, alkenylamines, cyclicamines or arylamines with (2) one member selected from the group consisting of alkylglycidylethers, cycloalkylglycidylethers, arylglycidylethers, alkenylglycidylethers, glycidylalkylates, glycidylalkenates and glycidylarylates.

\* \* \* \* \*

15

20

25

30

35

40

45

50

55

60

65